

Patented Dec. 18, 1951

2,578,790

# UNITED STATES PATENT OFFICE

2,578,790

## FROTH FLOTATION OF FERRUGINOUS IMPURITIES FROM FINELY DIVIDED GRANITE ROCK

James B. Duke, Medulla, Fla., assignor to Minerals Separation North American Corporation, New York, N. Y., a corporation of Maryland

No Drawing. Application May 7, 1951,  
Serial No. 225,064

20 Claims. (Cl. 209—166)

1

This invention relates to the removal of ferruginous impurities from finely divided granite rock; and the general object of the invention is to produce, from what are considered to be the waste materials of a granite rock industry, a material suitable for use in the glass and ceramic industries.

This application is a continuation-in-part of my co-pending application, Serial No. 100,539, filed June 21, 1949, now abandoned.

Granite, a crystalline igneous rock, is largely composed of quartz and feldspar; but, unfortunately for its usefulness in the glass and ceramic industries, it generally also contains ferruginous impurities such as biotite and hornblende, and in some cases minor amounts of iron containing garnet, muscovite, tourmaline, epidote, titanium, magnetite, hematite, etc. The particular object of the present invention is to remove the major portion of such ferruginous impurities from finely divided granite rock, by a method which is so simple and cheap that it is practicable for the production of a material that is saleable to the glass and ceramic industries. In its broader aspects the process of this invention may be utilized to remove ferruginous impurities from igneous crystalline rocks containing feldspar as a major mineral constituent, which may be in the form of orthoclase, microcline, plagioclase or a feldspathoid such as nepheline, nepheline syenite, sodalite, or any natural combination of these minerals.

Evidently, finely divided granite rock and so-called "glass sands" have characteristics so different that the known methods of removing ferruginous impurities from glass sands do not give as satisfactory results when applied to the treatment of finely divided granite rock. This fact became apparent when an effort was made to employ prior art methods for the removal of ferruginous impurities from finely divided granite rock from the vicinity of Tyrone, Georgia.

The method of the present invention is the result of the discovery that a useful material having a low iron content can be obtained economically by froth-floating the ferruginous impurities away from crushed granite, even in a single froth-flootation operation, after conditioning an aqueous pulp of the finely divided granite with cooperating flotation agents consisting of an unsaponifiable oil; a cationic-active nitrogenous compound of the kind hereinafter mentioned, an anionic-active fatty acid compound of the kind hereinafter mentioned, and a frothing agent. More specifically stated, the said method employs as the flotation agents an unsaponifiable oil; a cationic-active nitrogenous compound containing an aliphatic group which contains from 7 to 19 carbon atoms; an anionic-active fatty

2

acid compound having a hydrocarbon radical of at least 12 carbon atoms; and a frothing agent. It will be noted that neither a mineral acid nor an alkali is included among the cooperating flotation agents employed in the method of the present invention, in spite of the teachings of the prior art such as the U. S. Patent to Cole, Duke and McMurray 2,409,665. It is surprising that the agents above mentioned cooperate in such a way that satisfactory froth-floating of the ferruginous impurities takes place when a feed of finely divided granite rock is subjected to froth-flootation treatment.

The unsaponifiable oil may be (for example) fuel oil, lubricating oil, diesel oil, etc. Examples of the cationic-active nitrogenous compounds which have been found to be satisfactory include aliphatic amines and their salts, quaternary ammonium compounds, pyridinium compounds, phosphonamides, and imidazolines.

The aliphatic amines and their salts include, for example, the commercial product formerly sold by E. I. du Pont de Nemours and Company as "D. P. 243" which is understood to be a 50% aqueous paste of technical laurylamine hydrochloride containing approximately 18% octylamine hydrochloride, 10% decylamine hydrochloride, 55% laurylamine hydrochloride, 17% myristylamine hydrochloride and traces of secondary and tertiary amines; the commercial product sold by Armour and Company as "Am. Ac. 1180-C" which is understood to consist of approximately 73% mono-octadecylamine acetate, about 24% monoheptadecylamine acetate, together with small quantities of secondary and tertiary amine acetates; the commercial product of the Hercules Powder Company, known as "Rosin Amine Acetate" which is understood to be largely composed of the acetate of resin amines obtained from a modified rosin; the two commercial products of Armour & Co. known as "Armeen 12-D" which is understood to be a lauryl amine, and "Armeen 218" which is understood to be di-n-octadecylamine; and a product supplied by the Rohm & Haas Co. under the designation "Alkylamine JM" which is understood to be composed of tertiary-alkyl primary amines containing about 18 carbon atoms.

The quaternary ammonium compounds include, for example, two products of Armour & Co. known as "Arquad 18" which is understood to be octadecyl-trimethyl ammonium chloride, and "Arquad 12" which is described as dodecyltrimethyl ammonium chloride.

The pyridinium compounds include, for example, cetyl pyridinium chloride, and a product of the Emulsol Corporation known as "Emcol 888" which is understood to be largely composed of

a polyalkylnaphthalene methyl-pyridinium chloride.

As an example of phosphonamides, a product of the Victor Chemical Co. was used which is known as "Victamine D" which is understood to be the stearly amine salt of the stearyl-amide of ethyl phosphoric acid.

The imidazolines include, for example, two products of the Carbide & Carbon Chemical Corp. known as "Amine 22L" and "Amine 220" which are understood to be glyoxalidines of different molecular weights and the general structure:



wherein R represents an alkyl or alkenyl group containing from 10 to 20 carbon atoms; R<sub>1</sub> represents a hydrocarbon or a lower alkyl group; R<sub>2</sub> represents an alkylene group or a lower alkyl substituted alkylene group; and X represents a hydroxyl group, an amine group, or an amino-alkylene substitute imino group.

The fatty acid compound may be, for example, red oil (oleic acid), or a crude fatty acid compound derived from fish oil; or tall oil which is a liquid resinous oily by-product of the sulfite process used in paper making, which is a mixture of fatty and resin acids. As the frothing agent, pine oil may be employed.

The invention will be understood from the following description of examples of preferred methods of utilizing it for the removal of the major portion of the ferruginous impurities from finely divided granite rock, principally composed of quartz and feldspar. In Examples 1, 2 and 5, the cationic-active nitrogenous compound employed was D. P. 243, and the anionic-active fatty acid compound was red oil (oleic acid). In Example 3, the cationic-active nitrogenous compound employed was Am. Ac. 1180-C, and the anionic fatty acid compound was tall oil. In Example 4, the cationic-active nitrogenous compound employed was rosin amine acetate, and the anionic fatty acid compound was fish-oil fatty acid. Example 5 shows the highly satisfactory results when the invention is applied to an acid-treated feed.

#### Example 1

Granite rock, composed principally of orthoclase and silica with iron impurities in the form of biotite and hornblende and minor amounts of garnet, magnetite and hematite received from the vicinity of Tyrone, Georgia, was reduced to -10 mesh by crushing it in a laboratory jaw crusher. The -10 mesh portion was then screened on a 48 mesh screen and the +48 mesh portion was ground in a porcelain pebble mill to -48 mesh, and that ground material was added to the -48 mesh material resulting from said screening. Then the -48 mesh material thus obtained was mixed with water and deslimed on a 325 mesh screen by decantation. The deslimed ground feed thus obtained was conditioned in an aqueous pulp with the reagents (hereinafter mentioned) at about 70% solids for about two minutes and was then subjected to froth-flotation treatment, thereby producing a froth product rich in iron minerals which was discarded, and a machine discharge low in iron minerals which was the final product. The reagents employed, in lbs. per ton of feed, were as follows: D. P. 243, 0.4 lb.; fuel oil, 3.0 lbs.;

red oil (oleic acid), 0.7 lb.; and pine oil 0.9 lb. The metallurgical results were as follows:

| Products               | Per Cent Wt. | Per Cent Fe | Distribution, Per Cent Fe |
|------------------------|--------------|-------------|---------------------------|
| Feed.....              | 100.0        | 1.61        | 100.0                     |
| Froth Product.....     | 39.3         | 3.9         | 95.5                      |
| Machine Discharge..... | 60.7         | 0.12        | 4.5                       |

#### Example 2

The same granite rock was reduced to -10 mesh in a laboratory jaw crusher. The -10 mesh portion was mixed with water and then screened on a 35 mesh screen. The +35 mesh portion was ground for about 11 minutes in an aqueous pulp at about 50% solids in a porcelain pebble mill. The pebble mill discharge was screened on a 35 mesh screen, and the -35 mesh fraction was added to the primary -35 mesh fraction. The +35 mesh fraction was reground in the pebble mill for about 5½ minutes and screened on a 35 mesh screen; and the oversize was ground by hand to -35 mesh and added to the -35 mesh above mentioned. This gave a -35 mesh feed which was mixed with water and then deslimed by decantation on a 200 mesh screen. A 500 gram charge of the deslimed -35 material thus obtained was then conditioned in an aqueous pulp at about 70% solids for about two minutes, with the same reagents in the same quantities as those used in Example 1. The fuel oil was added to the pulp while the agitator in the conditioner was still; and the other agents were added while the agitator was moving. The time of conditioning began when the last of the reagents had been added. The thus conditioned feed was then subjected to froth-flotation treatment, which produced a froth product rich in iron minerals which was discarded, and a machine discharge low in iron minerals which was the final product. The metallurgical results were as follows:

| Products               | Per Cent Wt. | Per Cent Fe | Distribution, Per Cent Fe |
|------------------------|--------------|-------------|---------------------------|
| Feed.....              | 100.0        | 1.63        | 100.0                     |
| Froth Product.....     | 44.9         | 3.48        | 95.5                      |
| Machine Discharge..... | 55.1         | 0.127       | 4.3                       |

#### Example 3

In this example, the crushed and ground granite rock feed was prepared in the same way as in Example 2. The feed was then conditioned with the agents (hereinafter mentioned) in the same manner as in Example 2, but different cationic and anionic reagents were employed, the reagents, per ton of solids in the feed, being: Fuel oil, 3.0 lbs.; Am. Ac. 1180-C, 0.4 lb.; tall oil, 0.7 lb.; and pine oil 0.9 lb. The metallurgical results were as follows:

| Products               | Per Cent Wt. | Per Cent Fe | Distribution, Per Cent Fe |
|------------------------|--------------|-------------|---------------------------|
| Feed.....              | 100.0        | 1.66        | 100.0                     |
| Froth Product.....     | 49.8         | 3.20        | 95.9                      |
| Machine Discharge..... | 50.2         | 0.134       | 4.1                       |

#### Example 4

In this example, the feed was prepared in the same way as in Examples 2 and 3; and the agents

employed, per ton of solids in the feed, were fuel oil, 3.0 lbs.; Hercules rosin amine acetate, 0.4 lb.; fish-oil fatty acid 0.7 lb.; and pine oil 0.9 lb. The metallurgical results were as follows:

| Products          | Per Cent Wt. | Per Cent Fe | Distribution, Per Cent Fe |
|-------------------|--------------|-------------|---------------------------|
| Feed              | 100.0        | 1.62        | 100.0                     |
| Froth Product     | 38.4         | 4.04        | 96.0                      |
| Machine Discharge | 61.6         | 0.106       | 4.0                       |

From the foregoing Examples 1, 2, 3 and 4 it will be evident that the method which is the present invention results in obtaining from granite rock containing (on an average) 1.63% iron, a purified product containing (on an average) only about 0.122% iron, with the final product averaging 56.9% of the weight of the feed.

*Example 5*

This example shows the beneficial results obtained by pre-treating the feed with sulfuric acid. The feed was prepared in the same way as in Example 2; and to a 500 gram portion of that feed in an aqueous pulp at about 60% solids, was added sulfuric acid in the amount of 10 lbs. per ton of feed. The pulp was then allowed to stand for about 18 hours, and was then washed substantially free of acid with distilled water. To this acid-treated feed in a stationary aqueous pulp at about 70% solids was added 3.0 lbs. of fuel oil. The pulp was then agitated, and to it during agitation was added, in the order about to be mentioned, D. P. 243, 0.4 lb.; red oil (oleic acid), 0.7 lb.; and pine oil, 0.9 lb.; all per ton of solids in the feed. Agitation of the pulp was continued for about two minutes, and then the thus conditioned feed was subjected to froth-flotation treatment. This resulted in a froth product, high in iron minerals, which was discarded; and a machine discharge which was the finished product. The metallurgical results were as follows:

| Products          | Per Cent Wt. | Per Cent Fe | Distribution, Per Cent Fe |
|-------------------|--------------|-------------|---------------------------|
| Feed              | 100.0        | 1.57        | 100.0                     |
| Froth Product     | 37.5         | 4.08        | 97.5                      |
| Machine Discharge | 62.5         | 0.069       | 2.5                       |

It is evident that by acid-treating the feed in the manner above described, before conditioning it with the agents, improved results were obtained in the final product.

The following Examples 6, 7 and 8 utilize the invention for the removal of ferruginous impurities from two different samples of feldspar rock from North Carolina and Tennessee, and a nepheline syenite (containing sodalite) from Canada. These examples demonstrate the utility of the process for beneficiating feldspar ores in general.

*Example 6*

A feldspar rock from the vicinity of Burnsville, North Carolina, was wet screened on 35 mesh and the +35 mesh portion was ground to pass 35 mesh in a porcelain pebble mill with flint pebbles. The ground feldspar was added to the -35 mesh screened product and the whole sample was then deslimed by squirting with water and decanting over a 200 mesh screen. A 500 gram charge of the -35 mesh deslimed feldspar was

55 pulped with water at 70% solids and conditioned for about 2 minutes with the following reagents (expressed as pounds of reagent per short ton of dry feed): 3.0 lbs. of fuel oil, 0.3 lb. of red oil, 0.2 lb. of D. P. 243, and 0.2 lb. of pine oil, in a manner similar to the procedure used in Example 2. The conditioned pulp was diluted to about 20% solids in a minerals separation air-flow flotation cell and subjected to froth flotation treatment. The froth product, which was rich in the iron containing minerals muscovite and garnet, was discarded; while the machine discharge was the low iron beneficiated product. The metallurgical results were as follows:

| Products          | Per Cent Wt. | Per Cent Fe | Distribution, Per Cent Fe |
|-------------------|--------------|-------------|---------------------------|
| Feed              | 100.0        | 0.414       | 100.0                     |
| Froth Product     | 39.8         | 0.94        | 90.3                      |
| Machine Discharge | 60.2         | 0.067       | 9.7                       |

*Example 7*

25 A second sample of orthoclase feldspar from Erwin, Tennessee, was all -48 mesh and was deslimed and further treated in exactly the same manner described in Example 6. The same quantities of the same flotation reagents were used, and the same froth flotation treatment produced the following metallurgical results:

| Products                   | Per Cent Wt. | Per Cent Fe | Distribution, Per Cent Fe |
|----------------------------|--------------|-------------|---------------------------|
| Feed                       | 100.0        | 0.263       | 100.0                     |
| Froth Product <sup>1</sup> | 14.1         | 1.68        | 88.9                      |
| Machine Discharge          | 85.9         | 0.034       | 11.1                      |

<sup>1</sup> Principally muscovite and garnet.

*Example 8*

35 A sample of feldspar of the nepheline syenite class, which consisted largely of nepheline with smaller amounts of albite and sodalite, was reduced to -35 mesh and deslimed in the manner described under Example 6. It was also conditioned with reagents and subjected to froth flotation as described in Example 6, except that the red oil was reduced to 0.2 lb. and the D. P.-243 was reduced to 0.1 lb. per ton of feed. The metallurgical results were:

| Products                   | Per Cent Wt. | Per Cent Fe | Distribution, Per Cent Fe |
|----------------------------|--------------|-------------|---------------------------|
| Feed                       | 100.0        | 3.57        | 100.0                     |
| Froth Product <sup>1</sup> | 51.2         | 6.36        | 91.2                      |
| Machine Discharge          | 48.8         | 0.64        | 8.8                       |

<sup>1</sup> Principally hornblende and biotite.

*Examples 9 to 18*

60 These examples serve to illustrate the wide variety of cationic-active nitrogenous compounds containing an aliphatic group of from 7 to 19 carbon atoms, which can be utilized in the method of this invention in cooperation with an unsaponifiable oil, an anionic-active fatty acid compound containing a hydrocarbon radical of at least 12 carbon atoms, and a frothing agent.

65 The feed in these examples was prepared in the following manner: Granite rock received from Tyrone Rock Products Company was screened on a 10 mesh screen, and the + mesh portion was then crushed and again screened on the 10 mesh screen. The -10 mesh granite rock

thus obtained was then screened on a 35 mesh screen, and the +35 mesh fraction was then ground in a pebble mill for about 30 minutes and screened on a 35 mesh screen. Six charges to the pebble mill were thus ground, and the combined oversize was reground for about 30 minutes in the pebble mill and was screened on a 35 mesh screen. The small amount of oversize from this screening was discarded; and the combined -35 mesh portion of granite rock thus obtained was deslimed by agitation in water and decantation on a 200 mesh screen. All of the pebble mill grinding was done with enough water to cover the pebbles. Equal portions of the -35 mesh deslimed granite rock thus obtained were used as the feed in each of these Examples. This feed, which contained about 1.55% Fe, was conditioned at about 70% solids for about two minutes with the agents about to be mentioned, and was then subjected to froth-flotation treatment in a minerals separation airflow flotation cell. The fuel oil was added to a stationary pulp, the balance of the reagents was added to a moving pulp; and the reagents were added in the order and in the quantities listed below:

| Reagents                                  | Lbs per ton of feed |
|-------------------------------------------|---------------------|
| Fuel oil.....                             | 3.0                 |
| Cationic-active nitrogenous compound..... | (1)                 |
| Red oil (oleic acid).....                 | 0.4                 |
| Pine oil.....                             | 0.9                 |

<sup>1</sup> See table below.

The froth-flotation treatments to which the conditioned feeds were subjected in these Examples 9 to 18 produced froth products rich in iron minerals, and machine discharges low in iron which were the final products. In the interest of brevity, the metallurgical results of these examples are listed below in tabular form:

| Example No. | Cationic-Active Nitrogenous Compound | Lbs. | Machine Discharge |             |                    | Froth Prod., Per Cent Fe |
|-------------|--------------------------------------|------|-------------------|-------------|--------------------|--------------------------|
|             |                                      |      | Per Cent Wt.      | Per Cent Fe | Distr. Per Cent Fe |                          |
| 9.....      | Armeen 12D.....                      | 0.17 | 59.6              | 0.14        | 5.1                | 3.7                      |
| 10.....     | Armeen 218.....                      | 1.0  | 73.4              | 0.40        | 18.8               | 4.7                      |
| 11.....     | Alkylamine J. M.....                 | 0.4  | 82.4              | 0.30        | 15.9               | 7.5                      |
| 12.....     | Arquad 18.....                       | 0.2  | 42.8              | 0.21        | 5.9                | 2.5                      |
| 13.....     | Arquad 12.....                       | 0.15 | 56.7              | 0.18        | 6.7                | 3.2                      |
| 14.....     | Cetyl pyridinium chloride.....       | 0.1  | 76.2              | 0.28        | 13.3               | 5.7                      |
| 15.....     | Emcol 888.....                       | 0.4  | 46.3              | 0.19        | 5.7                | 2.8                      |
| 16.....     | Victamine D.....                     | 0.4  | 44.7              | 0.21        | 5.7                | 2.7                      |
| 17.....     | Amine 22L.....                       | 0.3  | 48.1              | 0.19        | 7.3                | 2.7                      |
| 18.....     | Amine 220.....                       | 0.35 | 53.0              | 0.19        | 6.8                | 2.9                      |

The results given in the above table show, in all the examples, the removal of substantial proportions of the iron from the feed of granite rock which contained (as hereinbefore mentioned) about 1.55% Fe. That is evidenced by the retention (as listed under "Distr. percent Fe") of only from 5.1% to 18.8% of this iron in the machine discharges which analyzed (as listed under "Machine Discharge percent Fe") much lower in percent Fe than the froth products. In contrast, a test on the same granite rock feed, omitting a cationic-active nitrogenous compound but using the other reagents in the same quantities, produced a machine discharge analyzing 0.9% Fe and representing 51.3% of the iron in the original granite rock feed.

What is claimed is:

1. The method of removing ferruginous im-

purities from materials of the feldspar and feldspathoid groups, which comprises conditioning an aqueous pulp of said finely divided material with cooperating agents consisting of an unsaponifiable oil, both a cationic-active nitrogenous compound containing an aliphatic group having from 7 to 19 carbon atoms and an anionic-active fatty-acid compound containing a hydrocarbon radical of at least 12 carbon atoms, and a frothing agent, and subjecting the thus conditioned pulp to a froth-flotation treatment thereby producing a ferruginous froth which is discarded, leaving the residue as the product which has a low iron content.

2. The method according to claim 1 in which the cationic-active nitrogenous compound is an aliphatic amine or salts thereof.

3. The method according to claim 2, in which the aliphatic amine salt is principally mono-octadecylamine acetate.

4. The method according to claim 1 in which the cationic-active nitrogenous compound is a quaternary ammonium compound.

5. The method according to claim 4, in which the quaternary ammonium compound is principally dodecyltrimethyl ammonium chloride.

6. The method according to claim 1 in which the cationic-active nitrogenous compound is a pyridinium compound.

7. The method according to claim 6, in which the pyridinium compound is principally a cetyl pyridinium chloride.

8. The method according to claim 1 in which the cationic-active nitrogenous compound is a phosphonamide.

9. The method according to claim 8, in which the phosphonamide is principally the stearyl amine salt of the stearyl amide of ethyl phosphoric acid.

10. The method according to claim 1 in which the cationic-active nitrogenous compound is an imidazoline.

11. The method of removing ferruginous impurities from finely divided granite composed principally of quartz and feldspar, which comprises conditioning an aqueous pulp of said finely divided granite with a mineral oil, both a cationic-active nitrogenous compound containing an aliphatic group having from 7 to 19 carbon atoms and an anionic-active fatty-acid compound having a hydrocarbon radical of at least 12 carbon atoms, and pine oil, and subjecting the thus conditioned pulp to a froth-flotation treatment thereby producing a ferruginous froth which is discarded, leaving the residue as the product which is a mixture of quartz and feldspar having a low iron content.

12. The method according to claim 11 in which the cationic-active nitrogenous compound is an aliphatic amine or salts thereof.

13. The method according to claim 12 in which the aliphatic amine salt is principally mono-octadecylamine acetate.

14. The method according to claim 11 in which the cationic-active nitrogenous compound is a 5 quaternary ammonium compound.

15. The method according to claim 14, in which the quaternary ammonium compound is principally dodecyltrimethyl ammonium chloride.

16. The method according to claim 11 in which 10 the cationic-active nitrogenous compound is a pyridinium compound.

17. The method according to claim 16, in which the pyridinium compound is principally cetyl pyridinium chloride.

18. The method according to claim 11 in which the cationic-active nitrogenous compound is a phosphonamide.

19. The method according to claim 18, in which the phosphonamide is principally the stearyl amine salt of the stearyl amide of ethyl phosphoric acid.

20. The method according to claim 11 in which the cationic-active nitrogenous compound is an 25 imidazoline.

JAMES B. DUKE.

#### REFERENCES CITED

The following references are of record in the file of this patent:

#### UNITED STATES PATENTS

| Number    | Name           | Date           |
|-----------|----------------|----------------|
| 2,088,325 | Kirby          | July 27, 1937  |
| 2,267,307 | Ralston et al. | Dec. 23, 1941  |
| 2,288,237 | Greene         | June 30, 1942  |
| 2,337,118 | Lontz          | Dec. 21, 1943  |
| 2,352,324 | Hubler         | June 27, 1944  |
| 2,395,475 | Gibbs et al.   | Feb. 26, 1946  |
| 2,409,665 | Cole et al.    | Oct. 22, 1946  |
| 2,483,192 | Gieseke        | Sept. 27, 1949 |

#### OTHER REFERENCES

Bulletin of the American Ceramic Society, vol. 18, No. 8 (1939), "Froth Flotation of Talc Ores from Gouverneur, New York," by Norman et al., page 206.

Rock Products for December 1946, page 91, "Flotation Chemicals for Non-metallic Minerals," by J. A. Barr.